

## UNITED STATES PATENT OFFICE.

CORNELIUS HORACE KELLER, OF SAN FRANCISCO, CALIFORNIA, ASSIGNEE TO MINERALS SEPARATION NORTH AMERICAN CORPORATION, OF NEW YORK, N. Y., A CORPORATION OF MARYLAND.

## CONCENTRATION OF ORES.

No Drawing.

Application filed November 24, 1925. Serial No. 71,226.

This invention relates to the froth-flotation concentration of ores and is herein described as applied to the concentration of a complex ore with the aid of the salt of an acid containing a complex radicle having such a metal as iron in an anion group.

Such ores may be rich but of little commercial value unless the contained minerals can be individually collected in separate concentrates. Moreover, such ores often contain iron in addition to the more valuable minerals, and, for commercial purposes, it is often necessary to obtain concentrates relatively free from iron.

These and other useful results have been attained by the employment of various substances as auxiliaries to the usual mineral-frothing agents. One of the substances so employed is a salt of xanthic acid. Another is dixanthogen. According to the present invention an auxiliary substance may also be a salt of an acid containing such a metal as iron in an anion group. In the procedure herein described this auxiliary is employed to enhance the action of the first auxiliary. The process is herein illustrated as applied to the extremely refractory San Francisco Mines of Mexico silver-lead-zinc ore, and as carried out with potassium ferricyanide as the second auxiliary substance used with sodium xanthate, but under such conditions that dixanthogen is formed, as will herein-after appear.

The ferricyanides differ widely from other salts somewhat similar in name. They are practically non-poisonous, are commercially available in large quantities at a price low enough to make their use feasible in commercial flotation, and form well-defined crystals so that the pure salt is easily recognized.

Ore of San Francisco Mines of Mexico was ground in a ball mill for fifteen minutes with sodium sulphide used at the rate of a half pound per ton of ore. The resulting pulp with added water was agitated for five minutes in a spitzkasten subaeration machine to produce a lead-froth rougher concentrate. This agitation was conducted with the addition of 3 pounds soda ash, 0.8 pound potassium ferricyanide, 0.04 pound sodium xanthate, 0.3 pound Barrett No. 634 oil, and 0.15 pound cresylic acid, all per ton of ore.

To the remaining pulp were added 0.5

pound sulphate of copper, 0.1 pound sodium xanthate, 0.3 pound Barrett No. 634 oil, and 0.2 pound steam distilled pine oil, all per ton of ore, and this pulp was then agitated ten minutes to produce a zinc-froth rougher concentrate.

The lead concentrate was then reagitated for three minutes with the further addition of 0.1 pound of cresylic acid per ton of original ore to form a finished lead concentrate and a lead middling.

The zinc concentrate was then reagitated for three minutes without any additional reagents to form a finished zinc concentrate and a zinc middling.

The results are shown in the following table:

|          | Wt.   | Ag.<br>(oz. per ton). | Assays. |      |      |
|----------|-------|-----------------------|---------|------|------|
|          |       |                       | Pb.     | Zn.  | Fe.  |
| Head.    | 100.0 | 27.8                  | 10.3    | 21.2 | 5.5  |
| Pb Conc. | 10.5  | 119.5                 | 67.0    | 10.0 | 3.0  |
| Pb Midd. | 7.8   | 74.2                  | 100.2   | 21.0 | 17.7 |
| Zn Conc. | 22.7  | 24.2                  | 3.5     | 27.5 | 11.1 |
| Zn Midd. | 6.2   | 21.3                  | 23.6    | 4.0  | 6.5  |
| Total.   | 82.8  | 5.2                   | 0.8     | 7.4  | 4.2  |

|          | Ag.   | Pb.   | Zn.   | Fe.   |
|----------|-------|-------|-------|-------|
| Head.    | 100.0 | 100.0 | 100.0 | 100.0 |
| Pb Conc. | 45.0  | 68.0  | 5.0   | 5.5   |
| Pb Midd. | 20.9  | 15.5  | 9.6   | 18.2  |
| Zn Conc. | 19.8  | 8.7   | 57.5  | 27.3  |
| Zn Midd. | 4.6   | 2.9   | 9.5   | 2.0   |
| Total.   | 9.7   | 2.9   | 18.4  | 42.0  |

It will be noted that the finished lead concentrate and the finished zinc concentrate are well above smelters' requirements and that even the middlings mixed with their respective finished concentrates meet such requirements. Also the silver appears to a very large extent in the lead concentrate where it is most valuable. Besides all this a very large proportion of the iron has been rejected and gone into the tailings.

It has been found that when equimolecular proportions of potassium ferricyanide and sodium xanthate are agitated together with the xanthate in such proportions and with an agitation such as are employed in the froth-flotation process, they react to form dixanthogen and probably ferrocyanide of potassium. In the proportions of the ex-

ample above given, however, there is a large excess of potassium ferricyanide over such equimolecular proportions and apparently although the sodium xanthate is converted into dixanthogen (the latter being a substance which will assist the action of a mineral-frothing agent) there is a considerable amount of potassium ferricyanide still present after this reaction. Potassium ferricyanide is a well known oxidizing agent.

Having thus described one embodiment of my invention what I claim is:

1. The process of concentrating ores which consists in agitating a suitable pulp of an ore with a mineral-frothing agent and with a xanthate and a substance containing an anion group including a metal adapted to react with the xanthate and produce a substance to cooperate with the mineral-frothing agent to produce a mineral-bearing froth containing a large proportion of a mineral of the ore, said agitation being so conducted as to form such a froth, and separating the froth.

2. The process of concentrating ores which consists in agitating a suitable pulp of an ore with a mineral-frothing agent and with a xanthate and a ferricyanide which react and produce a substance adapted to cooperate with the mineral-frothing agent to produce a mineral-bearing froth containing a large proportion of a mineral of the ore, said agitation being so conducted as to form such a froth, and separating the froth.

3. The process of concentrating ores which consists in agitating a suitable pulp of an ore with a mineral-frothing agent and with a xanthate and an excess of a substance which in part reacts with the xanthate to produce another substance and which is itself a substance containing a complex radicle containing iron both of which substances are adapted to cooperate with the mineral-frothing agent to produce a mineral-bearing froth containing a large proportion of a mineral of the ore, said agitation being so conducted as to form such a froth, and separating the froth.

4. The process of concentrating ores which consists in agitating a suitable pulp of an ore with a mineral-frothing agent and with a xanthate and with an excess of a substance containing a metal in the anion group which in part reacts with the xanthate to produce another substance and which is itself a substance containing a complex radicle containing iron both of which substances are adapted to cooperate with the mineral-frothing agent to produce a mineral-bearing froth containing a large proportion of a mineral of the ore, said agitation being so conducted as to form such a froth, and separating the froth.

5. The process of concentrating ores which consists in agitating a suitable pulp of an

ore with a mineral-frothing agent and with a xanthate together with an oxidizing substance adapted to cooperate with the mineral-frothing agent to produce a mineral-bearing froth containing a large proportion of a mineral of the ore, said agitation being so conducted as to form such a froth, and separating the froth, reagitating the remainder of the pulp with the further addition of flotation agent and separating another froth containing a large proportion of another mineral of the ore.

6. The process of concentrating ores which consists in agitating a suitable pulp of an ore with a mineral-frothing agent and with a ferricyanide adapted to cooperate with the mineral-frothing agent to assist in the production of a mineral-bearing froth containing a large proportion of a mineral of the ore, said agitation being so conducted as to form such a froth, separating the froth, reagitating the remainder of the pulp with the further addition of flotation agent and separating another froth containing a large proportion of another mineral of the ore.

7. The process of concentrating ores which consists in agitating a suitable pulp of an ore with a mineral-frothing agent and with a xanthate and an excess of a substance which in part reacts with the xanthate to produce another substance and which is itself a substance containing a complex radicle containing iron both of which substances are adapted to cooperate with the mineral-frothing agent to produce a mineral-bearing froth containing a large proportion of a mineral of the ore, said agitation being so conducted as to form such a froth, separating the froth, reagitating the remainder of the pulp with the further addition of reagents and separating another froth containing a large proportion of another mineral of the ore.

8. The process of concentrating ores which consists in agitating a suitable pulp of an ore with a mineral-frothing agent and with a xanthate of an alkali metal and a ferricyanide so as to produce a mineral-bearing froth containing a large proportion of a mineral of the ore, and separating the froth.

9. The process of concentrating ores which consists in agitating a suitable pulp of an ore with a mineral-frothing agent and with a xanthate of an alkali metal and a ferricyanide so as to produce a mineral-bearing froth containing a large proportion of a mineral of the ore, separating the froth, reagitating the remainder of the pulp with the further addition of flotation agent, and separating another froth containing a large proportion of another mineral of the ore.

In testimony whereof, I have affixed my signature to this specification.